

# UNITED STATES PATENT OFFICE.

JÖRGEN ERNST THOMSEN, OF JERSEY CITY, NEW JERSEY, ASSIGNEE TO THE JOSEPH DIXON CRUCIBLE COMPANY, OF JERSEY CITY, NEW JERSEY, A CORPORATION OF NEW JERSEY.

## ELECTRODE AND PROCESS OF MAKING THE SAME.

1,243,009.

Specification of Letters Patent.

Patented Oct. 16, 1917.

No Drawing.

Application filed February 2, 1917. Serial No. 146,204.

To all whom it may concern:

Be it known that I, JÖRGEN ERNST THOMSEN, a citizen of the United States, residing in Jersey City, in the county of Hudson, in the State of New Jersey, have invented certain new and useful Improvements in Electrodes and Processes of Making the Same, of which the following is a specification.

My invention relates to electrodes or electrical conductors and particularly to that class of electrodes which are composed partly of carbon. An object of my invention is to produce a harder and stronger article of this class than those in common use at present. Electrodes of my invention are of particular value as dynamo brushes, but they have numerous other uses.

In order that my invention may clearly be understood, I will describe in detail a specific embodiment of it.

In producing my electrode, I first mix together finely divided carbon, a phenol or creosol or a compound or mixture containing phenols and creosols, such as pitch, tar or creosote oil, and formaldehyde or a formaldehyde derivative, such as para-formaldehyde, and hexamethylenetetramin. I find it preferable not to have the carbon content of this mixture reduced to a uniform degree of fineness. It should preferably consist of particles of graphite of different sizes. If formaldehyde is used, I find it desirable also to add a small quantity of alkali, as, for example, ammonia, to the mixture.

The strength of the final material as well as its electrical conductivity may be varied by varying the proportion of the carbon to the other ingredients in the mixture. One formula which I have found to give a very satisfactory product is as follows:

64% carbon (containing particles of different sizes),

18% coal tar,

45. 15% creosote,

3% hexamethylenetetramin.

The above described mixture is then heated to a temperature not exceeding 450° F. to drive off the volatile matter and the remaining mass is ground to a powder.

The powder thus formed is then pressed into molds at a pressure which must vary according to the hardness and density desired in the product. When making the

electrode for use as a motor brush, I find 55 a pressure of two tons per square inch satisfactory.

The molded blocks are then calcined at a temperature above the decomposition points of the condensation products of the formaldehyde and the phenols and creosols. It is necessary to surround or cover the blocks with fine carbon during the calcining or otherwise prevent oxygen from coming in contact with the blocks when heated about 65 a red heat. In calcining, the temperature must be raised very slowly up to the point where the condensation products of the formaldehyde and the cresols and phenols are 70 fully carbonized and all the gases from their decomposition have been expelled. When this point is reached, the calcination is complete and a further increase in the temperature has no effect.

I wish it clearly understood that my invention is by no means limited to the specific embodiment which I have described. My invention is defined in the following claims, in which I have used the word "tar" 75 in a generic sense to include either wood tar, 80 coal tar or a mixture of the two or any substance or substances containing phenols or creosols or both.

I claim:

1. An electrode consisting of a hard non-inflammable body produced from a mixture of carbon, tar, and a compound containing the formaldehyde radical.

2. An electrode consisting of a hard non-inflammable body produced from a mixture 90 of finely divided carbon including particles of different sizes, tar, and a compound containing the formaldehyde radical.

3. An electrode consisting of a hard non-inflammable body produced from a mixture 95 of the following components in about substantially the following proportions: carbon 64%, tar 33%, and formaldehyde derivative 3%.

4. An electrode consisting of a hard non-inflammable body produced from a mixture of finely divided carbon containing particles of different sizes, phenols and creosols, and a compound containing the formaldehyde radical.

5. A process of making electrodes, comprising mixing together carbon, tar, and a compound containing the formaldehyde

100

105

- radical, pressing the mixture into blocks, and calcining the blocks at a temperature above the decomposition point of the condensation products present.
- 5 6. A process of making electrodes, comprising mixing together finely divided carbon containing particles of different sizes, tar, and a compound containing the formaldehyde radical, pressing the mixture 10 into blocks, and calcining the blocks at a temperature above the decomposition point of the condensation products present.
- 15 7. A process of making electrodes, comprising mixing carbon, tar, and a compound containing the formaldehyde radical, heating the mixture sufficiently to drive off the volatile matter, pressing the mixture into blocks, and calcining the blocks at a temperature above the decomposition point of the condensation products present.
- 20 8. A process of making electrodes, comprising mixing together carbon, tar, and a compound containing the formaldehyde radical, heating the mixture sufficiently to drive off the volatile matter, grinding the 25 resulting mass to a powder, pressing the powder into blocks, and calcining the blocks at a temperature above the decomposition point of the condensation products present.
9. A process of making electrodes, comprising mixing together finely divided carbon about 64%, tar about 33%, and formaldehyde derivative about 3%, heating the mixture to a temperature not exceeding 450° F. to drive off the volatile matter, grinding 30 the resulting mass to a powder, pressing the powder into blocks, and calcining the blocks at a temperature above the decomposition point of the condensation products present.

JÖRGEN ERNST THOMSEN.